

Sept. 7, 1926.

1,599,147

H. SCHMIDT ET AL

DUPLEX BLUE PRINT PAPER

Filed Sept. 4, 1923

Fig. 1.



Fig. 2.



Fig. 3.

INVENTORS  
Henry Schmidt  
William F. Kleb  
BY  
Marvin Bellin  
ATTORNEY

## UNITED STATES PATENT OFFICE.

HENRY SCHMIDT AND WILLIAM P. KLEB, OF RICHMOND HILL, NEW YORK.

## DUPLEX BLUE-PRINT PAPER.

Application filed September 4, 1923. Serial No. 680,901.

This invention relates to improvements in blue print paper, the main object being to produce a duplex paper having sensitized surfaces susceptible to stripping or separation after exposure and subsequent fixing, whereby two prints are attained by a single operation.

Another object is to provide an unusually effective formula for preparing the sensitized solution, with which the paper is permeated to a suitable extent, and also for the fixing bath used to set the prints, rendering them substantially permanent.

These objects are attained by the novel use of a duplex or layered fabric, as paper, treated chemically by the process as described in detail.

In the production of paper a relatively thin light weight web or sheet is superposed on the surface of the base sheet, each having been separately calendered and then passed together through other press rolls, causing them to remain in adherence until forcibly separated when dry.

This duplex paper is then treated by applying a sensitizing solution to the thin layer, saturating the same and permitting the lower thicker layer to become surface coated.

In the drawing, Figure 1 is a plan view of a sheet of the duplex paper showing a conventional print on its face, and Figure 2 is a view of the same sheet, the front layer being partially separated from the base.

These views show clearly that the print is disclosed on the base sheet, as well as on the thinner outer sheet, thus producing two prints at one operation.

Figure 3 is a fragmentary perspective view of the duplex paper, showing the double layers in close proximity.

Referring more in detail to the drawing:—

The numeral 10 designates any desired design on the top layer 11 of the sensitive paper. As the top layer is peeled off, the

design appears on the lower layer 12, as at 13, shown in Figure 2 of the drawing.

The solution for sensitizing blue print paper is made as follows:—

First, dissolve in five liters of hot water, 50 four thousand grams of ferrous sulfate crystals, nine hundred grams citric acid and add enough water to make ten liters of liquid.

Second, in five liters of hot water dis- 55 solve one thousand grams of potassium ferro cyanide, fifty grams potassium bichromate and add enough water to make ten liters.

When ready to apply take five parts of the first solution, two parts of the second 60 solution and three parts pure cold water.

The paper may be passed with the thin sheet downward through the mixture or it may be applied with a brush and after dry- 65 ing is in condition for exposure, in the usual manner.

After exposure the paper is thoroughly washed, preferably in running water, to remove all traces of the uncombined chemicals and dried.

Thereafter the thin sheet can be peeled or raised from the base sheet, and it will be noticed that the outside of the thin sheet presents a negative print on both sides, a similar negative appearing on the adjacent 75 face of the lower or base sheet.

Having thus described our invention what we claim as new and desire to secure by Letters Patent, is:—

As a new article of manufacture, a duplex 80 blue print paper comprising a relatively thin outer sheet saturated by a sensitizing solution, and a heavy base sheet coated on its exterior with the solution, both sheets being coalesced by pressure and readily sepa- 85 rable when in a dry condition.

In witness whereof we have signed our names to this specification.

HENRY SCHMIDT.  
WILLIAM P. KLEB.